

H. P. MACDONALD,  
METHOD OF AND APPARATUS FOR HEAT TREATING METALLIC ARTICLES.  
APPLICATION FILED FEB. 4, 1919.

1,335,977.

Patented Apr. 6, 1920.



WITNESS:

Prof R. R. Hitchcock.

INVENTOR

Harry P Macdonald  
BY  
Symington & Lechner  
ATTORNEYS

# UNITED STATES PATENT OFFICE.

HARRY P. MACDONALD, OF MONTCLAIR, NEW JERSEY, ASSIGNOR TO THE SNEAD & CO. IRON WORKS, OF JERSEY CITY, NEW JERSEY, A CORPORATION OF NEW JERSEY.

## METHOD OF AND APPARATUS FOR HEAT-TREATING METALLIC ARTICLES.

1,335,977.

Specification of Letters Patent.

Patented Apr. 6, 1920.

Application filed February 4, 1919. Serial No. 274,922.

*To all whom it may concern:*

Be it known that I, HARRY P. MACDONALD, a citizen of the United States, residing at Montclair, county of Essex, and State of New Jersey, have invented certain new and useful Improvements in Methods of and Apparatus for Heat-Treating Metallic Articles, of which the following is a specification.

10 This invention relates to an improved method of and apparatus for heat treating metallic articles, particularly tubing.

In general respects, the apparatus I employ in carrying out my invention is the same as that shown in United States Letters Patent to Macdonald and Huggins, No. 1,274,919. The apparatus shown in such patent comprises in the main, a vertical frame carrying an upper and a lower pair 20 of contact jaws adapted to receive the tube to be treated, the tube being suspended in vertical position and being discharged, after heat treatment, into an oil or other quenching bath located at the foot of the frame.

25 I have found that it is frequently necessary to give each piece of tubing three different heats in order to obtain the desired properties in the finished tube. In the first heat the tube is brought to the point of decalescence and is then quickly cooled or quenched. It is then again heated to the decalescent point, cooled, and finally re-heated to the drawing temperature and set aside to cool slowly.

35 It will be seen, therefore, that in the type of apparatus described, a considerable amount of additional work and a loss of time was entailed, owing to the fact that after the first heat, it was necessary to discharge the tube into the bath, remove it from the bath, replace it in the machine, where it was reheated and again discharged, to be again removed from the bath and replaced in the machine, and then, after re-heating to the drawing temperature, set aside for cooling.

40 It is the purpose of my present invention to overcome the foregoing difficulties and to provide an improved method and apparatus whereby the heat treating operations can be carried out expeditiously and with a minimum number of operations.

45 I accomplish the foregoing, together with such other objects as may hereinafter appear, by means of a construction which I

have illustrated in preferred form in the accompanying drawings, wherein:

Figure 1 is a diagrammatic side elevation of the main supporting frame with its tube supporting contacts, and with the means for 60 quenching the tube, while in the machine, in position to be placed in operation; Fig. 2 is an enlarged section through a portion of the tube with the quenching means, illustrating the position of the quenching 65 means at the end of a quenching operation; and Fig. 3 is a broken-away side elevation and partial section of a modified form of quenching means.

In carrying out my invention I provide, 70 as in the aforesaid Letters Patent, a vertically disposed main frame A, on which is mounted an upper pair of contact jaws B and a lower pair of contact jaws C, so arranged that the tube 7 to be treated is supported in vertical position with freedom to expand during the heating and cooling operations, the lower pair of jaws C being movable for this purpose by reason of the fact that its holding bolts pass through 80 elongated slots in the frame (see dotted lines Fig. 1). Current is passed through the tube by means of the leads 8 and 9, and the tube is heated by its internal resistance to the passage of the current.

85 In treating the tube, the operator first turns on the current and heats the tube to the decalescent point, which he may determine in any one of a number of different ways, and when this point is reached, the 90 current is turned off. Instead of then discharging the tube, in the manner shown in said patent, I leave the tube in the machine and lower into it a quenching element 10 preferably in the form of a pipe, closed at 95 the bottom and provided with a plurality of apertures 11 extending through the wall thereof. The pipe is supplied with oil, cold air, gas, or other quenching medium from a suitable source of supply 12 to 100 which the pipe 11 is connected by a flexible hose 13, the supply of quenching medium being controlled by the valve 14. The pipe 11 is preferably lowered into the tube, and upon, or just previous to, introduction of 105 the pipe into the tube, the valve 14 is opened and the quenching medium is discharged through the apertures 11 in such manner as to impinge substantially uniformly upon the entire inner surface of the tube.

After the tube has been quenched the pipe 11 is removed, current is again turned on, and the tube again brought to the decalescent point, after which it is again quenched 5 in the manner described, when the pipe 11 is withdrawn and the tube heated to the drawing temperature, whereupon it is removed from the machine and set aside to cool slowly. In some cases, it may not be 10 necessary to give the second heat.

The modification shown in Fig. 3 is particularly adapted for use where the quenching medium is cold air, although this form of quenching apparatus may also be employed 15 with other quenching mediums. It differs from the apparatus just described in that the pipe 11<sup>a</sup> is open only at the bottom end where it is provided with a cone-like jet member 15, which is adapted to discharge 20 the quenching medium in a laterally directed substantially uniform spray. With this construction, however, the valve 14 is opened just before or at the time the end of the pipe is introduced, and the pipe is lowered 25 at a uniform speed. Depending upon the treatment desired, it may be necessary to raise and lower the pipe several times throughout the length of the tube before the valve is closed.

It will be seen from the foregoing that I 30 have provided an apparatus for applying the quenching medium internally and this is advantageous not only because it makes it unnecessary to remove the tube from the 35 machine for the various operations, but also because the internal application of the quenching medium can be made more uniformly than an external application, and in addition, the quenching medium is more 40 effective.

Furthermore, it will be seen that the quenching medium is entirely under the control of the operator and the tube may be cooled to any desired point necessary. This 45 effects a saving in current for the reason that the operator, after the tube has been quenched, and while it is still hot, can switch on the current and start the reheating, whereas when the tube is dropped into an 50 oil bath, it acquires the temperature of the bath and sufficient current has to be used on the subsequent heatings to raise it from that temperature to the temperature desired for the treatment. The use of cold air for 55 a quenching medium is most advantageous in this respect.

I have found the foregoing process to be particularly valuable in the treatment of tubing such as referred to in the aforementioned Letters Patent in which the wall of 60 the tube is relatively thin. An example of such tubing specified in the said Letters Patent is a tube about ten feet long, an inch

in diameter with a thickness of wall of about one-sixteenth of an inch. It will be seen 65 that with such material in which the thickness of the wall is relatively such that the heating and quenching are accomplished with great speed considerable difficulties are encountered in heat treatment, particularly 70 with reference to the securing of the proper physical conditions throughout the metal.

I claim:

1. The herein described process of heat treating metallic articles which consists in 75 heating the article in suitable supporting mechanism; and in quenching the article, in reheating the article before cooling, in quenching the article, and in reheating the article to drawing temperature, *in situ*. 80

2. The herein described process of heat treating metallic tubing, which consists in heating the tube in suitable supporting mechanism by passing an electric current therethrough; and in quenching the tube 85 *in situ*; in again reheating the tube by passing the electric current therethrough before the tube has cooled; and in cooling the tube.

3. The herein described process of heat treating metallic tubing, which consists in 90 heating the tube in suitable supporting mechanism by passing an electric current therethrough; in quenching the tube *in situ* at the critical point; in again reheating the tube to the critical point by passing the current of electricity therethrough; in quenching the tube *in situ* at the critical point; and in again reheating the tube by passing the current of electricity therethrough to 95 a drawing temperature. 100

4. The herein described process of heat treating relatively thin tubing having a substantially uniform diameter and a substantially uniform thickness of wall which consists in simultaneously and uniformly heating all portions of the tube, and in simultaneously quenching the tube throughout its length by applying a quenching medium to the interior thereof substantially uniformly. 105

5. In the heat treatment of hollow metallic articles, the step which consists in simultaneously and uniformly heating all portions of the article by passing an electric current therethrough, and in uniformly applying a quenching medium in the interior 110 of the article *in situ*. 115

6. In the heat treatment of hollow metallic articles, the step which consists in simultaneously and uniformly heating all portions of the article by passing an electric current therethrough, and in substantially uniformly applying a gaseous quenching medium in the interior of the article *in situ*. 120

In testimony whereof I have hereunto signed my name.

HARRY P. MACDONALD.